

March 26, 1974

TAKEO HARADA

3,799,771

ELECTRICAL CONTACT MATERIAL CONTAINING SILVER, CADMIUM

OXIDE, TIN AND NICKEL

Filed Dec. 6, 1971

*FIG. 1*



*FIG. 2*



*FIG. 3*



3,799,771

**ELECTRICAL CONTACT MATERIAL CONTAINING SILVER, CADMIUM OXIDE, TIN AND NICKEL**  
 Takeo Harada, Mishima, Japan, assignor to P. R. Mallory & Co. Inc., Indianapolis, Ind.  
 Filed Dec. 6, 1971, Ser. No. 205,255  
 Int. Cl. C22c 5/00

U.S. CL. 75-178 A

15 Claims

**ABSTRACT OF THE DISCLOSURE**

Electrical contact material is disclosed containing silver, cadmium oxide, tin and nickel having a microstructure of cadmium oxide particles dispersed in a silver matrix which are fine and fibrous. The fibrous structure generally occurs normal to the oxidized surface.

**BACKGROUND OF THE INVENTION**

The present invention relates to new and useful improvements in a silver-cadmium oxide electrical contact material used for electrical contacts.

In general, silver-cadmium oxide electrical contact materials are characterized by being more resistant to sticking and resistant to erosion than silver electrical contact material, and the contact resistance is stable, so they are used widely for light current loads and medium-heavy loads.

Such silver-cadmium oxide electrical contact materials are manufactured by a powder metallurgical process, by a post oxidation process, or by a preoxidation process. The powder metallurgical process is a process in which a moulded mixture of silver powder and cadmium oxide powder is sintered, as described in greater detail, for example in U.S. Pat. 2,145,690. The post oxidation process comprises preparing a silver-cadmium alloy, working it to desired shape and heating it in oxidizing atmosphere so as to have cadmium thereof selectively internal oxidized. Further information may be found in U.S. Pats. 2,539,298 and 2,673,167. The pre-oxidation process, described in U.S. Reissue Pat. 27,075 and U.S. Pat. 3,545,067 involves forming fine particles of silver-cadmium alloy, for example by atomizing a melt of silver-cadmium alloy, internally oxidizing the cadmium in the particles, consolidating the oxidized particles and mechanically working to desired shape.

However, silver-cadmium oxide electrical contact materials are often unsatisfactory in regard to resistance to erosion and in breaking characteristics.

Therefore an object of the present invention is to provide an improved electrical contact material having a lower erosion rate. Another object of the present invention is to provide a contact material having improved hardness.

Another object of the invention is to provide a contact material having improved hardness at elevated temperature.

Another object of the present invention is to provide a contact material having lower sticking power.

Another object of the invention is to provide a contact material which has a stable contact resistance.

Other objects will be apparent from the following description and drawings wherein:

FIG. 1 is a photomicrograph of the microstructure of the electrical contact material of the present invention at 200 magnifications, containing 13% CdO, 1.0% Sn and 0.02% Ni.

FIG. 2 is a photomicrograph of the microstructure of post oxidized prior art contact material and containing silver cadmium oxide at the same magnifications as FIG.

1 and having the same cadmium oxide compositions as the material of FIG. 1.

FIG. 3 is a photomicrograph of electrical contact material of the prior art containing, silver, cadmium oxide and tin at the same magnifications as FIG. 1 with the same composition of cadmium oxide and tin as the material of FIG. 1.

**SUMMARY OF THE INVENTION**

- 10 The electrical contact characteristics of silver-cadmium oxide electrical contact material are improved by adding about 0.2 to about 5% tin and about 0.005 to 0.5% nickel to the material. The microstructure comprises fine and fibrous grains of cadmium oxide precipitated in a silver matrix.
- 15 Preferably the material contains about 0.3 to 2% tin and about 0.01 to 0.3% nickel.

**DETAILED DESCRIPTION OF THE INVENTION**

- 20 The present invention relates to an electrical contact material manufactured by oxidizing a silver-cadmium alloy prepared by adding 0.2 to 5% tin (weight % and hereinafter in this application) and 0.05 to 0.5% nickel to silver-cadmium to provide a material consisting essentially of up to 30% cadmium, about 0.2 to about 5% tin, about 0.005 to about 0.5% nickel, the balance silver. The addition of tin has the effect of causing the configuration of the grains of cadmium oxide during selective oxidation to be a fibrous structure normal to the oxidized surface as shown in FIG. 3. The added amount of tin under 0.2%, however, does not make the effect of the addition distinguishable and an amount over 5% increases the precipitation of cadmium at the grain boundary, reducing the electrical conductivity and workability of the alloy considerably. Preferably the tin content is from about 0.3 to about 2%.

- 25 The addition of nickel is effective in causing the grains of cadmium oxide after the internal oxidation of the silver-cadmium alloy to be remarkably fine as can be seen from comparing FIGS. 1 and 3. The cadmium oxide particles are generally not larger than  $1\mu\phi \times 10\mu$ . The added amount of nickel under 0.005% does not make the effect of the addition distinguishable. Nickel, however, is only slightly solid soluble in silver and cadmium, so its added amount is not above about 0.5%. Preferably the nickel content is from about 0.01 to about 0.3%. The preferred material consists essentially of about 5 to about 15% cadmium, about 0.3 to about 2% tin, about 0.01 to about 0.3% nickel, the balance silver.

- 30 The electrical contact material of the present invention may be manufactured for example by either the post-oxidation or pre-oxidation techniques mentioned above.

- 35 In regard to the pre-oxidation technique, U.S. Reissue Pat. 27,075 and U.S. Pat. 3,545,067 are hereby incorporated into the present application by reference and may be referred to for exemplary processing parameters which may be used in processing according to this technique.

- 40 In utilizing this technique the nickel and tin may be added to the silver melt prior to atomizing. An excess of tin and nickel may be added to allow for any losses of tin and/or nickel while adding these elements to the melt and/or during pouring.

- 45 The tendency for the fibrous structure to appear normal to the oxidized surface is often lost in this technique. While the fibrous structure is normal to the oxidized surface within individual particles, since these particles are randomly consolidated and are subsequently mechanically worked, the fibrous structure becomes random throughout the microstructure.

- 50 In regard to the post oxidation technique, U.S. Pats. 2,539,298 and 2,673,167 are hereby incorporated into the

present application by reference for their description of exemplary temperature ranges and other processing parameters which may be used in processing according to this technique. The tendency for the fibrous structure to be normal to the oxidized surface is greater when this technique is used than with the pre-oxidation technique because the oxidation step occurs after the article has been formed so that the tendency for the fibrous structure to be normal to the oxidation face is not lost through consolidation of oxidized particles and/or mechanical working to shape.

In general, in oxidizing the fine particles according to the pre-oxidation technique, or the finished or semi-finished shape according to the post-oxidized technique, an oxidation temperature of about 700 to about 850° C. and a time of about 5 to about 150 hours is preferred, depending upon section size, oxidizing temperature, and oxygen content of the atmosphere.

The hardness of the electrical contact material is greater than prior art material of similar cadmium oxide composition without nickel. It is really at least about 50% higher at room temperature and is often twice as hard. The hardness at elevated temperature is also improved at least about twice and is usually as hard as prior art material of similar cadmium oxide composition.

Also the arc erosion rate and sticking power are lower with the material of the present invention. The arc erosion rate is usually at least 25% lower and often 50% or more lower. The sticking is usually at least 50% lower and is often three times lower.

#### SPECIFIC EMBODIMENTS

An alloy comprising 13.3% cadmium oxide, 0.45% tin oxide, 0.03% nickel oxide and the balance silver is manufactured by adding 12.0% cadmium, 0.5% tin, and 0.5% nickel to a silver melt and rolling the resulting casting to sheet form having a thickness of 1.5 mm. and then heating it at 700° C. for 96 hours in an oxygen containing atmosphere. The electrical conductivity and hardness of said silver-cadmium oxide alloy are shown in Table 1, together with those of another alloy as a comparative material prepared under the same conditions as above by adding 13.3% cadmium oxide to silver.

TABLE 1

| Sample | Electrical conductivity, IACS, percent | Hardness, HRF |
|--------|----------------------------------------|---------------|
| A----- | 56                                     | 71            |
| B----- | 68                                     | 40            |

NOTE.—A=The contact material according to the present invention. B=The comparative material.

The hardness of the contact material according to the present invention is about twice as large as that of the comparative material, because the addition of tin and nickel causes the grains of cadmium oxide to be fine and fibrous.

The results of the erosion test carried out with the contact material according to the present invention and the comparative material respectively, each having the shape of a contact having the size of 7 mm. x 7 mm. x 1.2 mm. incorporated in a 35 ampere frame electromagnetic switch are shown in Table 2.

TABLE 2

| Sample | Eroded amount (mg.) after 500,000 times of switching | Contact resistance (mΩ) after 500,000 times of switching |
|--------|------------------------------------------------------|----------------------------------------------------------|
| A----- | 900                                                  | 7.5                                                      |
| B----- | 1,700                                                | 10.0                                                     |

NOTE.—A=The contact material to the present invention. B=the comparative material.

Test conditions:

Voltage: 200 v.

Current:

at making, 47 A., pf. 0.35

at breaking, 235 A., pf. 0.65

Switching frequency: 20 time/min.

Moreover, the results of the stick test carried out with the contact material according to the present invention and the comparative material respectively each in the shape of the contact having the diameter of 6 mm. and the thickness of 1.5 mm. are shown in Table 3.

TABLE 3

| Sample | Number of times of switching | Sticking power (kg.) | Eroded amount (mg.) |
|--------|------------------------------|----------------------|---------------------|
| A----- | 10                           | 1.3                  | 6.5                 |
| B----- | (1)                          | 12.0                 | 32.0                |

<sup>1</sup> Stuck at 7th time.

<sup>2</sup> Determined when contact stuck at 7th time of switching.

NOTE.—A=The contact material according to the present invention.

B=The comparative material.

Test conditions:

Voltage: 100 v.

Current: 2000 A.

Contact pressure: 200 g.

Closing time: 2 cycles

Closing frequency: 10

The eroded amount of the contact material according to the present invention is about half that of the comparative material (not added with tin and nickel) as shown in Table 2, and Table 3 shows that the sticking power of the former is about one-ninth of that of the latter in the stick test under the current 2000 A. Therefore, the contact material according to the present invention has improved antierosive and antisticking properties.

As shown above, the silver-cadmium oxide electrical contact material according to the present invention is industrially very favorable due to its improved contact characteristics.

What is claimed is:

1. Ag-CdO type electrical contact material having improved hardness and erosion rate, the material consisting essentially of an effective amount up to 30 wt. percent Cd, about 0.2 to about 5 wt. percent Sn, about 0.005 to about 0.5 wt. percent Ni, and the balance Ag, the material being oxidized to convert oxidizable constituents to their respective oxides prior to use as an electrical contact material.

2. The Ag-CdO type electrical contact material of claim 1, wherein the Cd content is from about 5 to about 15 wt. percent, the Sn content is about 0.3 to about 2 wt. percent, and the Ni content is about 0.01 to about 0.3 wt. percent.

3. The Ag-CdO type electrical contact material of claim 1, wherein the microstructure of the contact material comprises CdO grains in an Ag matrix in which CdO grains are fine and fibrous.

4. The Ag-CdO type electrical contact material of claim 3, wherein the fibrous structure of the CdO grains is substantially normal to the oxidized surface of the contact material.

5. The Ag-CdO type electrical contact material of claim 4, wherein the CdO particle size is not generally larger than  $1\mu\phi$  x  $10\mu$ .

6. The Ag-CdO type electrical contact material of claim 2, wherein the Sn content is greater than about 0.5 wt. percent but less than about 2 wt. percent.

7. A method of making the Ag-CdO type electrical contact material of claim 1 comprising the steps of providing a melt of Ag-Cd-Sn-Ni to form a body consisting essentially of an effective amount up to 30 wt. percent Cd, 0.2 to 5 wt. percent Sn, 0.005 to 0.5 wt. percent Ni, the balance Ag, and subjecting the body to oxidation to

convert oxidizable constituents to their respective oxides and form the contact material, the Sn and Ni constituents cooperating to cause grains of CdO to be fine and fibrous.

8. The method of claim 7, including the further step of causing grains of CdO to be substantially normal to the oxidized surface of the contact material.

9. The method of claim 7, wherein the body is subjected to oxidation prior to forming a contact shape.

10. The method of claim 8, including the further step of forming the body into a cast shape having the thickness of the contact material prior to subjecting the cast shape to oxidation.

11. The method of claim 8, wherein the CdO particle size is about  $1\mu\phi \times 10\mu$  or less.

12. The method of claim 10, wherein Cd-Sn-Ni are 15 added to a melt of Ag.

13. A method of making the Ag-CdO type electrical contact material of claim 2 comprising the steps of forming an Ag melt, adding to the Ag melt Cd-Sn-Ni to form

a body consisting essentially of 5 to 15 wt. percent Cd, 0.3 to 2 wt. percent Sn, 0.01 to 0.3 wt. percent Ni, the balance Ag, subjecting the body to oxidation to convert the oxidizable constituents to their respective oxides, and causing the grains of CdO to be fine and fibrous and normal to the oxidized surface thereby forming the electric contact material.

14. The method of claim 13, wherein the CdO particle size is about  $1\mu\phi \times 10\mu$  or less.

15. The method of claim 14, wherein the Sn is more than about 0.5 wt. percent but less than about 2 wt. percent.

#### References Cited

#### UNITED STATES PATENTS

3,607,244 9/1971 Kabayama et al. 75—173 R

L. DEWAYNE RUTLEDGE, Primary Examiner

E. L. WEISE, Assistant Examiner

UNITED STATES PATENT OFFICE  
CERTIFICATE OF CORRECTION

Patent No. 3,799,771 Dated 03/26/74

Inventor(s) Takeo Harada

It is certified that error appears in the above-identified patent and that said Letters Patent are hereby corrected as shown below:

Col. 1, line 28, delete current after light.  
Insert current after medium-heavy.

Col. 2, line 23 delete--0.05 after and  
insert--0.005--

Col. 2, line 27 delete--0.005 after about  
insert--0.05--

Signed and sealed this 5th day of November 1974.

(SEAL)  
Attest:

MC COY M. GIBSON JR.  
Attesting Officer

C. MARSHALL DANN  
Commissioner of Patents